

# UNITED STATES PATENT OFFICE.

ROBERT FULTON TOMPKINS, OF NEW YORK, N. Y., ASSIGNOR TO THE BINDER COMPANY,  
A CORPORATION OF NEW JERSEY.

## COHERING OR BINDING COMPOSITION FOR ROADS OR OTHER PURPOSES AND ROADS OR PATHS COMPRISING THE SAME.

1,214,972.

Specification of Letters Patent. Patented Feb. 6, 1917.

No Drawing.

Application filed August 15, 1913. Serial No. 734,884.

To all whom it may concern:

Be it known that I, ROBERT FULTON TOMPKINS, a citizen of the United States, residing at New York, in the county of New York and State of New York, have invented certain new and useful Improvements in Cohering or Binding Compositions for Roads or other Purposes and Roads or Paths Comprising the Same, of which the following is 10 a specification.

This invention relates to binding compositions for substances of divided or separated nature, such as sand or insoluble silicious or silicon containing material, or other substance of mineral, vegetable, or animal nature, and such materials bonded thereby.

The object of the invention is to provide an efficient binder of vegetable nature and of carbon compound character comprising a 20 glucosid, a glucosid and tannin, and either or both associated with a water solvency retardant, such as resinous materials or substances capable of forming the same like rosin oil, which rosin oil I prefer to employ, 25 and has for certain specific applications the property of binding, securing or anchoring road-dust together in such a manner that its circulation by air currents occasioned by moving vehicles or other means is limited or 30 prevented and whereby a solid compact and hardened road-bed and road dressing is produced and an automatic hygroscopic coherence or adherence created, without materially injuring or destroying the coherer or 35 adhering binder, and also for binding molders' sand or composition for cores, etc., for gluing, sizing, or cementing of cellular or cellulose containing material or products or fabrications thereof, such as paper, paste- 40 board, straw board, and the like, and for other purposes.

One species of the composition included in the present invention comprises glucosids of the aromatic extractive type, such as glucosid tannins which appear in tanning extracts or products, in proportion of about 45 27 per cent. by weight together with tannin 21 per cent. and water 52 per cent., which composition has an approximate gravity of 50 forty-eight degrees Twaddell, associated with a resinifying substance such as rosin oil.

This product or composition may be produced by concentrating the spent tan liquors

containing approximately 2 per cent. of glucosid and tannin in approximate proportion to each other by weight as one and a half to one, or an aqueous solution of 2 degrees Twaddell, by evaporation or dehydration to a density of 48 degrees Twaddell, and adding thereto 2 per cent. of rosin oil.

To this composition of glucosid or tannin containing rosin oil may be added a soluble silicate such as sodium silicate in proportion of 5 per cent. by weight of the combined glucosid and tannin content when the binder is intended to be employed as a street or road dressing or as a cement or glue for paper, straw or other cellulose containing substances or fabrication.

The advantages of this binder, comprising glucosids and tannin together with a water solvency resistant resides in the fact that when applied to paper or other cellulose substances which are matted or bonded by glues or sizes of glue nature, that the glucosid tannins and other tannins act as a glue or binder while they simultaneously fix the glue or size bonding material in the paper or other cellulose fabrication making a practically water repelling seal or binding, while the glucosid present is just sufficiently hygroscopic to prevent the drying out of the material to a point of brittleness thus producing a substantially water-repellent and flexible or resilient gluing medium. The soluble sodium silicate, when employed, also augments the adhering of the composition and maintains a flexibility which does not occur when substances comprising the silicate alone, as in the prior art, are employed.

When the binder is employed as a road dressing or binder, the tannin or tannic acid combines with the iron, alumina, lime or other constituents of the road construction material producing water insoluble compounds which present to the glucosids and other ingredients of the binder a superior adhesive surface so that the glucosids and excess tannins act as an agglutinating agent 100 for anchoring or securing particles of dust or other material together in a fixed and flexible or elastic manner while the inherent hygroscopic properties of the glucosids provides a ready and automatic moistening constituent and effect without deliquescence so that the particles adhere together without becoming attached to foreign materials 105

which may contact them such as vehicle tires, etc., while the rosin oil oxidizes and resinifies and acts to turn the water and retard the solvency of the ingredients in water.

5 The glucosids employed may be of any selective character, they being compounds which combine the properties of glucose and vegetable extractives, or what may be termed glucose esters, in such a manner that 10 each has lost its specific physical identity as such and is less soluble than either individually in water as a rule, and is hygroscopic, without deliquescence and does not effloresce or dry up spontaneously. The peculiarly adaptable properties or qualities of 15 these glucosids probably is attributable to a progressive and alternate hydrolysis into vegetable extractives or organic or carbon-containing acids and glucose and its reformation of glucosids by condensation and dehydration under atmospheric conditions of 20 heat, moisture and pressure.

The resinous material or substance capable of forming the same such as rosin oil 25 augments the cementing or anchoring quality of the composition, especially when associated with insoluble silicates, silicious, or silicon containing substances such as are usually found associated with or form a 30 part of road construction and at the same time increases the water repellent nature of the product.

The composition of tannin and glucosids 35 may be produced by mixing the individual ingredients with water or secured from such substances as spent tan liquors, or from other sources, or extracted from natural derivatives, or artificially or synthetically prepared, and rosin oil associated or combined 40 therewith.

Some of the tannins and tannic acids are at once so called tannins and glucosids, they being converted by hydrolysis into glucose and gallic, ellagic, protocatechuic and other 45 acids or organic extractives.

The composition comprising glucosids and tannins together with water, such as may be obtained from or as spent tan liquors, or fluid tan waste products such as are ordinarily thrown away, either as such, or products which may be obtained by boiling down 50 or concentrating the same, or such concentrated product rediluted combined with rosin oil, is particularly adaptable to road 55 treatment, acting as it does to fix the dust and cement the road base thus maintaining a form of fixed binder which is continually working its way into and between particles or pieces of the road construction when subjected at intervals to progressive watering 60 either by artificial sprinkling or from the natural source of rain, etc. It also exhibits the further enhancing quality of presenting a latent form of moisture by reason of its 65 hygroscopic properties thus preventing the

disintegration and drying out or crumbling of the road dressing or base body, and also provides a superior dressing or binding agent for construction materials of roads or other solid vehicle or transportation bearing body or path.

This material applied to the surface of such roads as asphalt roads or pathways, and then coated or sanded with frictional substances, has the property of anchoring or 75 securing such material to the asphalt surface thereby preventing the slipping of horses or skidding of vehicle wheels, the astringent properties of the tannin ingredients augmenting the frictional surface of 80 the road as presented to contacting substances such as vehicle tires, and also presents the additional feature of holding and securing or anchoring frost and ice to the roadway in such a manner that it is not 85 easily released under pressure and forms a foothold of frictional character for horses' shoes and the like, thus avoiding the usual dangerous character presented when ice is formed upon water repellent surfaces such 90 as asphalt, which results in slipping under pressure through the release of the unanchored ice coating.

This dust cohering and roadway cementing fluid has the advantage over oil dressings in that it does not injure or destroy 95 rubber tires of vehicles or affect the varnish of the same injuriously, nor is it lost by evaporation, nor does it affect injuriously metal, wood or leather, or reduce the gravity 100 of the road dressing so that it is floated and washed away by water or give a greasy appearance or dull coating to varnish or contents of vehicles.

When this binding or cementing material 105 comprising glucosids, or glucosid and tannin, combined with a resinous or resinifying substance such as rosin oil is employed as a binding or cementing agent in road construction forming a road base, it is mixed 110 with a sufficient proportion of such ordinary ingredients as broken stone, sand, gravel and the like, after any ordinary well-known fashion and then the whole mixed with suitable mineral cementitious or other 115 uniting or binding substances, such for instance as cement, forming a concrete, and the composition spread, rolled, tamped or otherwise placed in proper position or location whereby it will become set or fixed in 120 composite form.

The road bed, when it has been properly provided as aforesaid, is spread with a top dressing of granulated or finely divided material of mineral nature associated with the 125 glucosid, and rosin oil, or glucosid, tannin and rosin oil and the same rolled in and allowed to set, thus forming a compact dressing of water repellent nature and sufficiently of water absorbent character to retain the 130

moisture and prevent drying out and dusting of the composition and producing a compact and resilient blanket composition.

Instead of a cement concrete base containing the binder as aforesaid having a direct top dressing of the character described, the material of the road bed may be primarily dressed with an asphalt composition upon which a top dressing or finish of the character described is placed in communication with the asphalt layer, comprising sufficiently granulated or comminuted frictional substances, such as sand in such a manner that the frictional substances are anchored to, cemented by, or united with the surface of the asphalt coating.

Some of the advantages of a road of this character over roads constructed hitherto resides in the fact that the comminuted particles of the road produced by wear and tear during use by tires of vehicles and the like, are held together by the natural binding or cementing character of the material present and prevented largely from dusting by circulation in currents of air actuated by the movement of vehicles and the withdrawing of fine particles of the road bed by suction of the vehicle tread, the moisture occluded or held in the hygroscopic water repellent binder being displaced under pressure by the vehicle weight upon it, catches and secures any associated fine material in juxtaposition thereto, and holds the same to the contacting material and thereafter when the elastic binder recovers or resumes its original volume by expansion re-absorbs and retains the same.

The action of heat on a road bed or road of the character of the present invention does not have the effect of destroying the cohering and adhering properties of the binding or cementing ingredients of non-volatile character with retaining moisture, as is the case where oils are employed which are of more or less dry or volatilizable character, nor does the binder destroy or injure the surface of asphalt roads or the tires of vehicles.

Instead of mixing the binder directly with the constituents of the road construction during the road building, it may be applied to the road or roadway after the same is constructed, by sprinkling a sufficiently fluid solution upon the road and allowing it to soak in and preferably rolling the same thereafter to form a compact top dressing, and this mixture when sprinkled upon or otherwise applied to the road surface, is allowed to soak in and is preferably subjected to a second sprinkling or wetting by a slightly more dense binder consisting of approximately one part of concentrated material to two of water, the interval of time between the two applications being sufficient to allow the first coat to be absorbed or

combined in such a manner as to act both as a cementing agent and as a leader or path for the more dense liquor to be absorbed, and for the purpose of rolling and setting to be accomplished; the proportion of the first sprinkling liquor being approximately one of the binder to three of water.

Asphalt roads or roadways may be dressed with frictional substances, such as sand, bonded or united with binding compositions, in accordance with the present invention, of hygroscopic nature, and it will hold down the dressing against the flow of water over the impermeable asphalt containing surface, the dressing being thus retained or anchored to the asphalt will largely enhance the friction of the road surface under pressure, or attrition and retard the slipping of horses' shoes and the skidding of vehicle tires, the slipping and skidding of which presents one of the greatest difficulties and objections to the ordinary asphalt top dressing *per se*, and it also provides a means for anchoring sheeted particles of ice, which may form on the road bed to the surface of the asphalt thereby increasing the utility of asphalt roads and preventing this other serious objection to their employment. The composite coating or dressing of mineral substances bonded by a binder in accordance with the present invention, also forms a gravity blanket comprising cohering and adhering particles when employed in conjunction with the roadbed of existing roads, railroads or other viaducts for vehicles or other purposes, whereby the cementitiously aggregated material is collectively retained against currents of air and the road bed protected against water and currents thereof removing the surface. This material spread upon such roads as asphalt roads, not only provides a superior surface of frictionable nature, but also protects the asphalt surface against wear and loss of volatile constituents, which is often occasioned by the action of the heat of the sun, thus prolonging the life and utility of such asphalt-containing roads.

Where oil alone is used to cause the coherence or adherence of particles in a road or road dressing, it is not only lost by evaporation and drying out, but it likewise reduces the gravity of the fine contacting particles of the road dressing so that water, from rain or other source, causes it to float and be carried off, oil also produces an injurious and disintegrating effect upon vehicle tires and greases and destroys the appearance of varnish and other finish upon vehicles, exerts a deleterious action on metal, wood and leather, as well as creating a greasy, dusty atmosphere, injurious to the eyes and clothes and which also settles in houses upon furniture and other contents in the vicinity and contaminates water upon

which it falls, such as contained in reservoirs and the like, and also forms a sticky contamination on clothes, which is hard to remove, all of which disadvantages are obviated by the employment of glucosids and a water resistant or glucosids in tannin and a water resistant as a binder in accordance with the present invention as binding or cementing agents as a road dressing and 5 they are of water resisting but water retaining character and form in conjunction with other materials, when cementing the same, as a mineral road dressing, and produce a substance of greater gravity or of 10 increasing gravity with relation to water, than oil, so that it is not so readily washed away, and at the same time maintains the road dressing in a naturally and progressively moist condition by taking up or absorbing moisture from the atmosphere automatically, to compensate for the moisture dislodged or dissipated by evaporation through the action of heat, such as the sun, etc., due to the binding or cementing constituent's inherent properties, of hygroscopic 15 nature.

The tannic acid employed may be applied as free acid either alone or associated with other vehicles, substances of fillers, or it may be derived from substances capable of yielding same by decomposition or dissociation either by action of the road bed constituents, or substances intended therefor, or other means at or prior to its association. Some 30 of the materials from which tannic acid may be derived may be noted as the glucosids which are ethereal salts or esters of tannic acid, or substances containing the same otherwise united, such as the materials 35 known as sulfite pulp waste, which carries aldehydes and ketones capable of forming and delivering tannic acid upon decomposition.

The term "tannin" as employed herein is 40 intended to imply and does imply and include substances of the tannin nature or character capable of presenting and exhibiting fiber fixing or collagen coagulating properties similar to tannic acid such as is 45 found and occurs in the so-called sulfite pulp waste *per se* or upon concentration and the present binding composition is intended to include substances of these various characters associated with water resistant substances of resinous or resinifying character 50 such as rosin oil.

Having now described my invention, what I claim as new and desire to secure by Letters Patent is:—

60 1. A cohering or binding composition for roads or other purposes, comprising a hy-

groscopic glucosid and a fixed water insoluble water resistant.

2. A cohering or binding composition for roads or other purposes, comprising an aromatic glucosid and a water resistant. 65

3. A cohering or binding composition for roads or other purposes, comprising a hygroscopic glucosid and a water insoluble resinous substance. 70

4. A cohering or binding composition for roads or other purposes, comprising an aromatic glucosid and a resinous substance.

5. A cohering or binding composition for roads or other purposes, comprising a glucosid and a fixed oil. 75

6. A cohering or binding composition for roads or other purposes, comprising an aromatic glucosid and an oil.

7. A cohering or binding composition for roads or other purposes, comprising a glucosid and rosin oil. 80

8. A cohering or binding composition for roads or other purposes, comprising an aromatic glucosid and rosin oil.

85 9. A road or path, comprising a silicious substance, bonded by a composition comprising a glucosid and a water resistant.

10. A road or path, comprising a silicious substance, a glucosid, and a resinous material. 90

11. A road or path, comprising a silicious substance, bonded by a composition comprising a glucosid, and an oil.

12. A road or path, comprising a silicious substance, a glucosid and rosin oil. 95

13. A cohering or binding composition for roads or other purposes, comprising tannin and rosin oil.

14. A cohering or binding composition for roads or other purposes, comprising the concentrated or dehydrated constituents of spent tan bark liquor and a water resistant. 100

15. A cohering or binding composition for roads or other purposes, comprising the constituents of spent tan bark liquor and a water resistant. 105

16. A cohering or binding composition for roads or other purposes, comprising the concentrated or dehydrated constituents of spent tan bark liquor and rosin oil. 110

17. A cohering or binding composition for roads or other purposes, comprising the constituents of spent tan bark liquor and rosin oil. 115

In testimony whereof I affix my signature in presence or two witnesses.

ROBERT FULTON TOMPKINS.

Witnesses:

WM. J. JULIEN,  
JOHN HENRY HURLBULL.